

## UNITED STATES PATENT OFFICE

2,028,349

LUBRICANT AND PROCESS OF MAKING  
SAME

Mathias Pier, Heidelberg, and Friedrich Christmann, Ludwigshafen-on-the-Rhine, Germany, assignors to I. G. Farbenindustrie Aktiengesellschaft, Frankfort-on-the-Main, Germany

No Drawing. Application June 28, 1933, Serial No. 678,054. In Germany July 1, 1932

## 3 Claims.

(Cl. 87—9)

The present application is a continuation in part of our application Ser. No. 651,802, filed January 14th, 1933, in which a process is described and claimed according to which substances valuable for lubricating purposes, in particular as lubricants themselves or as additions to lubricants, are prepared by condensing waxy substances rich in hydrogen, in particular paraffin wax or substances containing the same, 10 by voltolization, i. e. by treatment with silent electric discharges.

According to a specific embodiment of the invention described and claimed in the said application the said substances obtained by voltolization are very useful when added to lubricants in conjunction with other additional agents. Thus lubricants containing hard or soft paraffin wax, especially lubricating oils, gear oils, lubricating greases and gear greases are much improved by 20 adding thereto small amounts of high molecular hydrocarbons which, even in small amounts, increase the viscosity and also such voltolization products as are capable of lowering the setting point.

25 We have now found that the aforesaid advantages obtained by adding to the said lubricants containing hard or soft paraffin wax, in particular to hydrocarbon oils boiling above 325° C. and containing hard or soft paraffin wax, small amounts of high molecular hydrocarbons which, even in small amounts, are capable of increasing the viscosity and also voltolization products capable of lowering the setting point, are not restricted to the said voltolization products, but that 35 instead of these voltolization products also other substances capable of lowering the setting point can be added with like advantage in conjunction with products capable of increasing the viscosity to the said oils containing hard or soft paraffin 40 wax.

45 As products capable of lowering the setting point mainly come into question, besides the said voltolization products, the substances obtainable by condensation of high molecular hydrocarbons rich in hydrogen, in particular hard or soft paraffin wax or substances containing the same, such as petrolatum or of paraffins having a molecular weight of more than 350, preferably in the presence of cyclic hydrocarbons, as described in our 50 copending application Ser. No. 480,284, filed September 6th, 1930 or by condensation of oxygen derivatives of aliphatic hydrocarbons or high molecular weight as described in our copending application Ser. No. 666,542, filed April 17th, 55 1933. The additions exerting effects in the dif-

ferent directions, namely increase in the viscosity and lowering of the setting point, are not mutually injurious and in most cases the setting point, which is not influenced or only slightly influenced by the additions increasing the viscosity when added alone, is still further improved and the viscosity index favorably influenced. These effects are astonishing, since if substances lowering the setting point are added in like amounts to different oils having different viscosities, the setting point is lowered the less the more viscous is the oil to be improved. This reduction in the effect of lowering the setting point is not observed with oils, the viscosity of which has been increased by the addition of substances having this particular effect.

As oils containing paraffin wax which are to be improved according to the present invention may be mentioned especially those which have a high flashpoint, as for example Mid-Continent 20 oils, Pennsylvanian oils, lubricating oils still containing hard or soft paraffin wax obtained by destructive hydrogenation, or oils containing paraffin wax which have been treated with liquefied hydrocarbons which are gaseous at room temperature, with phenols, with sulphur dioxide or with other solvents or extraction agents.

In order to increase the viscosity and improve the temperature-viscosity curve, hydrocarbons having a molecular weight of more than 1000, 30 preferably of more than 2000, are added to the said oils, these should have the property of exerting a favorable effect in this direction even when added in small amounts.

Substances suitable for this purpose are for 35 example the hydrocarbons having a high molecular weight of more than 1000, preferably of more than 2000, which are selected from the polymerization products of unsaturated hydrocarbons capable of forming polymeric homologous 40 series, and the products obtainable therefrom by hydrogenation, by isomerization, or by isomerization and hydrogenation, preferably those which on heating up to 200° C. for 5 minutes do not undergo appreciable decomposition, such 45 as hydrogenated rubber or hydrogenated polymerization products of diolefines, in particular butadiene, or cyclo rubber, or hydrogenated resins soluble in high-boiling oils, or polymerized styrene, or hydrogenated polymerized styrene, or 50 polymerized indene or oil-soluble polymerization products of olefines, such as isobutylene, preferably those which are prepared at low temperatures, if desired in the presence of volatile halides, or hydrogenated balata or gutta percha, or cellu- 55

lose derivatives, as for example cellulose laurate, and their hydrogenation products. These substances are added to the oils in an amount of from 0.5 to 10 per cent, preferably of from 1 to 5 per cent.

The substances lowering the setting point are added in a small amount, as for example from 0.5 to 10 per cent.

In the aforescribed manner oils can be obtained which have a low setting point and a viscosity index lying far above 100. Lubricating oils treated in the said manner may, by reason of their flat temperature-viscosity curves and their good mobility at low temperatures, be employed both in summer and in winter.

The following example will further illustrate the nature of this invention but the invention is not restricted to this example.

*Example*

1 per cent of a hydrogenated rubber and 1 per cent of a substance capable of lowering the setting point and prepared as described in Example 1 of the application Ser. No. 480,284 are added to a machine oil containing paraffin wax derived from German petroleum by distillation and having a viscosity index of 70, a viscosity of 1.8° Engler at 100° C. and a setting point of 3° C. The resulting mixture has a viscosity index of 107, a viscosity of 2.4° Engler at 100° C. and a setting point of 25° below zero centigrade.

If, instead of the hydrogenated rubber, 30 per cent of a natural or synthetic cylinder oil having a viscosity of from 8° to 10° Engler at 100° C. and a setting point of from 5° to 8° below zero centigrade, be added, the resulting mixture has the same viscosity, a viscosity index of about 100 and a setting point of only 17° below zero centigrade.

If instead of the said substance lowering the setting point 1 per cent of a volatilization product is added which is prepared as described in Example 1 of the said application Ser. No. 651,802 the same results are obtained. If 2 per cent of aluminium stearate is added as substance lowering the setting point the setting point of the said machine oil is reduced to 10° below zero centigrade in the case of the addition of 1 per cent of hydrogenated rubber and to 6° below zero centigrade when replacing the hydrogenated rubber by the aforesaid 30 per cent of natural or synthetic cylinder oil.

What we claim is:

1. A valuable hydrocarbon mixture essentially consisting of a lubricant containing paraffin wax

and containing a small amount of a hydrocarbon product having a mean molecular weight of at least 1000 and being capable of increasing the viscosity and flattening the temperature viscosity curve of hydrocarbon oils and being selected from the group consisting of the polymerization products of unsaturated hydrocarbons capable of forming polymeric homologous series, the products obtainable therefrom by hydrogenation, isomerization or isomerization and hydrogenation, hydrogenated rubber, hydrogenated resins soluble in high boiling oils, hydrogenated balata and hydrogenated gutta percha and a small amount of a substance different from the viscosity regulator capable of lowering the setting point of hydrocarbon oils and selected from the group consisting of high molecular weight volatilization products of waxy hydrocarbons rich in hydrogen, condensation products of paraffinic hydrocarbons having a high molecular weight, both per se and in conjunction with cyclic hydrocarbons, and condensation products of high molecular weight aliphatic oxygen-containing compounds.

2. A valuable lubricant essentially consisting of a lubricating oil containing paraffin wax and containing a small amount of a hydrocarbon product having a mean molecular weight of at least 1000 and being capable of increasing the viscosity and flattening the temperature viscosity curve of hydrocarbon oils and being selected from the group consisting of the polymerization products of unsaturated hydrocarbons capable of forming polymeric homologous series, the products obtainable therefrom by hydrogenation, isomerization or isomerization and hydrogenation, hydrogenated rubber, hydrogenated resins soluble in high boiling oils, hydrogenated balata and hydrogenated gutta percha and a small amount of a substance different from the viscosity regulator capable of lowering the setting point of hydrocarbon oils and selected from the group consisting of high molecular weight volatilization products of waxy hydrocarbons rich in hydrogen, condensation products of paraffinic hydrocarbons having a high molecular weight, both per se and in conjunction with cyclic hydrocarbons, and condensation products of high molecular weight aliphatic oxygen-containing compounds.

3. A lubricant according to the preceding claim in which the amount of each of the viscosity increasing and setting point lowering substances is from .5 to 10% of the lubricating oil.

MATHIAS PIER.  
FRIEDRICH CHRISTMANN.

CERTIFICATE OF CORRECTION.

Patent No. 2,028,349.

January 21, 1936.

MATHIAS PIER, ET AL.

It is hereby certified that error appears in the printed specification of the above numbered patent requiring correction as follows: Page 2, second column, lines 17 and 42, claims 1 and 2 respectively, for "volatilization" read voltolization; and that the said Letters Patent should be read with this correction therein that the same may conform to the record of the case in the Patent Office.

Signed and sealed this 25th day of January, A. D. 1938.

Henry Van Arsdale,

Acting Commissioner of Patents.

(Seal)